

W. A. CECIL.

PROCESS FOR PRESERVING WOOD.  
APPLICATION FILED SEPT. 25, 1916.

1,253,667.

Patented Jan. 15, 1918.

2 SHEETS—SHEET 1.



WITNESSES

W. C. Fielding  
Lloyd W. Patch

INVENTOR  
William A. Cecil

BY *Richard Oliver.*

ATTORNEY

W. A. CECIL,  
PROCESS FOR PRESERVING WOOD,  
APPLICATION FILED SEPT. 25, 1916.

1,253,667.

Patented Jan. 15, 1918.

2 SHEETS—SHEET 2.



WITNESSES

*W. C. Fielding*  
*Lloyd W. Patch*

BY *Richard A. Owen.*

INVENTOR  
*William A. Cecil*

ATTORNEY

# UNITED STATES PATENT OFFICE.

WILLIAM A. CECIL, OF EVANSVILLE, INDIANA, ASSIGNOR OF ONE-HALF TO ROBERT R. WILLIAMS, OF EVANSVILLE, INDIANA.

## PROCESS FOR PRESERVING WOOD.

1,253,667.

Specification of Letters Patent. Patented Jan. 15, 1918.

Application filed September 25, 1916. Serial No. 122,125.

*To all whom it may concern:*

Be it known that I, WILLIAM A. CECIL, a citizen of the United States, residing at Evansville, in the county of Vanderburg and State of Indiana, have invented certain new and useful Improvements in Processes for Preserving Wood, of which the following is a specification.

My invention relates to a new and improved method of preserving wood by impregnating the same with preservative fluids, and especially to a new and improved process for preserving railroad cross ties, pilings, structural and mine timbers, street paving blocks, etc., in which any preservative fluids may be used either singly or in admixture regardless of difference of specific gravities, while the pressure and the temperature of the fluids in the impregnating cylinder or retort are automatically controlled by means of a system of circulating pipes, and specially constructed automatically and mechanically operated valves which are so arranged that a uniform rise of pressure of the fluid in the impregnating cylinder is accomplished, this process being in part divisional matter from the application which eventuated into Patent No. 1,178,182, granted to me April 4, 1916.

As is well known, the heretofore generally used method of wood preservation by injecting chemical preservatives into the wood has consisted of placing the wood to be treated in a receptacle or retort capable of being closed air and liquid tight. If the wood be not sufficiently dry to permit of its thorough saturation without steaming, steam is admitted to the retort to accomplish the desired steaming and is maintained until the temperature attains the desired point, generally about 250 degrees Fah. This temperature is maintained until the wood is heated sufficiently to permit the moisture being drawn from the pores and cells thereof in the form of vapor, and by vacuum, a vacuum pump being coupled with the retort and started subsequent to the closing of the steam supply. This vacuum pump is operated until a vacuum equal to 22 to 25 inches of mercury at sea level is drawn, this vacuum being maintained for thirty minutes to one hour, or for any time that the operator judges necessary to draw a sufficient

amount of moisture from the wood to allow injection of the required volume of the preservative fluid.

Next, without admitting air to the retort or otherwise breaking the vacuum, the preservative fluid is admitted to the retort until the same is filled and all of the wood completely submerged. The outlet valves are maintained closed and more liquid is pumped into the retort so that the hydrostatic pressure in the retort is raised and thus the liquid forced into the wood. In some cases a separate closed tank or receiver is connected by a large pipe to the retort. The general practice has been to place this receiver so that when the retort is full of the fluid, the level of the fluid in the receiver or tank is somewhat below the top, thus leaving an empty space into which air is pumped under pressure. As the pressure of the air is increased the pressure upon the liquid is communicated from the closed tank or receiver through the connecting pipe to the fluid in the retort until the required pressure is attained in the retort; gages or recording instruments generally being provided to determine the exact working conditions, and the pressure being maintained until a sufficient amount of the preservative is forced into the wood.

In the use of the above outlined processes, there has never been any circulation of the preservative fluids in the retort except for the purpose of maintaining emulsions of more or less immiscible fluids, such as zinc, chlorid and creosote, but the liquids have in all cases been permitted to lie quiet and in a dead state in the retort while maintained under pressure. By this maintenance of the dead pressure within the retort, and through the consequent lack of movement and circulation of the fluid, the liquid or treating fluid varies in its temperature in the various parts of the retort, and especially in exposed locations the fluid becomes too cold for proper penetration, thus causing a different absorption of the fluid by the timber in different parts of the retort even when the timber is of the same species.

Further than this, to accomplish the most successful treatment of the timber, the pressure in the retort is to be raised at a uniform rate and the rapidity of increase of

pressure in the retort should only be such as will compensate for the increase of the resistance to the preservative fluid as the same penetrates into the wood and through 5 the gradual filling of the pores or cells thereof, the specification for treating timber generally requiring that the pressure in the retort shall be raised at a rate not to exceed 25 pounds per square inch in fifteen 10 minutes until the required maximum pressure is attained. To fulfil this requirement, it has heretofore been necessary for the operator to stand at the pump almost continually during the period of raising the pressure, and, at such times as he judged proper, to increase the pressure by increasing the speed of the pump, or where pneumatic pressure, instead of hydraulic, is used the pressure has been controlled by carefully 15 regulating the amount of air admitted to the air receiver, and then again under some circumstances the desired rises in pressure have been accomplished by bringing the pressure up in steps of 25 pounds at a time 20 and practically every fifteen minutes. All of these methods are unsatisfactory as they depend entirely upon the attention of and manual manipulation by the operator, and any neglect or failure to observe the niceties 25 of manipulation is conducive to erratic penetration. Also, it is under some circumstances required that preservative chemicals such as coal-tar creosote and refined coal-tar, coal-tar creosote and water gas tar, coal-tar creosote and water gas creosote, coal-tar creosote and crude oil, coal-tar creosote 30 and zinc chlorid solution, and etc, be used and except in the case of emulsions of creosote and zinc chlorid solutions, no attempt 35 has heretofore been made to assure perfect mixture of the preservative chemicals. As the result, it is by no means certain that the different ingredients will remain mixed in the proper solution so that the proper proportion 40 of each chemical will be carried into the pores of the wood but the natural tendency is for the chemicals to separate and for one chemical to have a better penetration than the remaining chemical or chemicals 45 of the solution, and here it might be set forth that the proper solution and an equal distribution of all of the ingredients throughout the entire volume of liquid which will insure a proper penetration of 50 the solution can be attained and maintained only by circulation.

Again, it is not possible to entirely exhaust the air from the cells of the wood and as the preservative fluid is forced into the 55 pores and cells of the wood this air is liberated as is also the air which is used in the mixture of the emulsions of preservative fluid, which are for the most part aerated mixtures, as the fluid is forced into the wood. 60 In all processes wherein dead pressures are

maintained or circulation is accomplished by means of a closed circuit apparatus, air must remain in the retort and it will of course be readily apparent that this presence of air in the retort is detrimental to 70 uniform absorption as it interferes with the homogeneity of mixtures of preservatives when circulation is maintained by means of closed circuit apparatus, and in some instances the volume of air may become sufficiently great to displace the fluid in the retort to such an extent that some of the wood on the top of the charge in the retort may not be entirely submerged at all times. 75

With the above in mind, it is a purpose of 80 my invention to overcome the above named and other faults of processes heretofore used, by employing a process which contemplates an open circuit circulation of the treating fluid and the automatic control of 85 the pressure of the preserving fluid, while at the same time permitting the use of mixtures and emulsions of preservatives of immiscible chemicals and maintain the same in the proper condition even though they be 90 aerated mixtures, allowing the successful use of the same by permitting the air from the mixtures and any air which may be forced out of the wood to escape.

It will be understood that a number of 95 variations might be resorted to in the apparatus to be employed in accomplishing my process, but I have endeavored to illustrate only one possible form which will permit the accomplishment of the various steps 100 of the treating action in the proper cycles and intervals.

In the drawings:

Figure 1 is a schematic view showing the retorts together with the liquid supply tank 105 and the circulating pipes to give the general arrangement of the parts of the apparatus, and with portions shown in vertical section.

Fig. 2 is a detail view to illustrate the automatic valve and to show one form of power and gear means which might be employed in the actuation of the same. 110

Fig. 3 is a view in elevation to better illustrate the structure shown in Fig. 2.

Fig. 4 is an enlarged detail sectional view to better illustrate the structure of the automatic pressure valves. 115

Fig. 5 is a detail view showing a dia- 120 phragm pressure switch which might be used in connection with an electric motor imparting movement to the mechanically operated valve and which switch will automatically stop the motor when the maximum pressure as desired is attained in the retort. 125

The liquid supply tank 1, which is designed to contain the supply of preservative liquid which is being constantly circulated through the retort 2 during the operation 130

of treating timber therein, has a suitable agitator located therein to keep the supply of liquid constantly agitated and mixed.

This agitator may be of any desired 5 form but in the present instance is illustrated as an air supply pipe 3, which is run to the bottom of the liquid supply tank 1, and is extended along the bottom thereof where it is provided with perforations as 10 indicated at 4, these perforations being preferably extended throughout the entire length of the portion of the pipe which is disposed adjacent to the bottom of the supply tank and to thus discharge air through substantially the entire volume of liquid and disturb 15 the ingredients of the greatest specific gravity which will have settled to the bottom of this tank, thus causing these ingredients to move in an upward current through the 20 ingredients of a least specific gravity which have a tendency to rise to the top of the mixture of fluid. By this arrangement of the parts, the entire body of fluid is constantly agitated and the desired mixture and homogeneity 25 of the same is maintained. It is obvious that this agitator will only be needed when the preservative fluid is composed of two or more preservatives of a more or less immiscible nature which are to be mixed to 30 form the preservative fluid, and I therefore desire to limit its use to the conditions under which it is needed.

The retort 2, will generally be of cylindrical form but may be of any desired shape 35 and of dimensions to suit the particular use, this retort being provided with one open end, and a door 5 being adapted to be closed over the open end and held liquid and air tight by securing bolts or clamps 6. 40 A fill and return pipe 7 connects with the bottom of the liquid supply tank 1, and at its opposite end is connected with the retort 2 at a point low down on the sides thereof. A suitable valve 8, preferably of the gate 45 type, is provided to control the opening through this pipe 7, and the pipe is intended only to accomplish the initial filling of the retort 2 after the timber to be treated has been placed therein and the door 5 has been 50 secured in place, and to permit the return of the preservative fluid from this retort when the treating action has ceased and it is desired to empty the retort so that the door 5 can be opened to permit the removal 55 of the treated timber and the placing of untreated timber in the retort to be impregnated.

A pressure pump 9 is installed as a part of the apparatus, and while I have herein 60 shown one specific form of pressure pump, and more particularly a pump of the piston type, I do not wish to limit myself to any particular pump but desire to have it understood that any kind of pump or any other suitable means which will supply liquid

under pressure may be used, the form of this part being that which appears to be more suitable for plant conditions under which it will operate. A pipe 10 extends from the lower part of the liquid supply 70 tank 1 to the pump 9, and a pipe 11 is connected from the pump to the retort 2, it being preferable that the pipe 11 be extended through the bottom of the retort 2 and that branch discharge pipes 12, each 75 provided with a plurality of openings 13, be connected with this pipe 11 to extend throughout the length of the retort 2 and to thus insure an even discharge of the liquid to all parts of the retort. A liquid 80 outlet pipe 14 has a plurality of branches and these branches are each connected with the retort 2 in the upper part thereof to thus permit discharge from the retort substantially uniformly from all parts thereof, an 85 automatic pressure valve 15 being connected in the discharge from the outlet pipe 14, and a return pipe 16 being connected with the automatic pressure valve 15 and led to the liquid supply tank 1 to thus allow discharge 90 of the liquid from the retort through the automatic pressure valve 15 and back to the liquid supply tank. A branch pipe 17 is connected to the outlet pipe 14 at one end, and at the opposite end this branch 95 pipe is connected with the return pipe 16, or the pipe 17 might be connected directly with the liquid supply tank to discharge into the bottom thereof, as local conditions might require. A mechanically operated 100 valve 18 having a specially constructed passage therethrough is mounted in this pipe 17 to control the passage of fluid therethrough and to consequently control the rate at which the liquid pressure in the retort 2 will be raised when this liquid is being constantly supplied by the pump 9, this regulation and control of the pressure being accomplished by a gradual throttling of the 105 passage through the valve.

A pipe 20 controlled by the valve 19 is connected in the pipe 11 at one end, and its opposite end is connected with the boiler supplying steam to the pump 9, or with any other suitable means to supply steam through 110 this pipe and through the plurality of openings 13 in the branch discharge pipe 12, the purpose of this steam being to dry the sap or other moisture out of the pores of the wood preparatory to the impregnating 115 process.

A pipe 21 is connected with the upper side of the retort 2, and a branch pipe 22 is connected with this pipe 21 and is extended to connect with any suitable source of compressed air supply, the valve 23 being provided to control the passage of fluid through this pipe 22. A second branch pipe 24, controlled by a valve 25, is connected with a vacuum pump or other suitable means which 120 125 130

may be set in operation to exhaust the fluid contents of the retort and to thus extract the moisture, air and steam from the retort, just prior to the introduction of the impregnating liquid thereinto.

The pressure control valve 18, as shown in detail in Figs. 2 and 3, may be a gate valve of the non-rising stem type with a passage through the same so proportioned 10 that when opened to its full extent substantially all the fluid discharged into the retort 2 by the pump 9 will pass through the valve when the pressure in the retort is so low as to not exceed five pounds above the pressure 15 due to elevation of the fluid in pipe 17. The valve 18 has a substantially triangularly shaped passage 28 therethrough, and the stem 29 by which the gate member is moved adjacent this triangularly shaped opening 20 or passage is screw threaded into the casing so that as the stem is turned, the gate member will be extended over or withdrawn from the passage. A relatively large worm gear 30 is connected on this stem 29 and a 25 transmission shaft 31 has a worm 32 mounted thereon to mesh with the worm gear 30. A worm gear 32 is carried on the opposite end of the transmission shaft 31 and a motor 33 has a worm 34 on the shaft thereof meshing with this worm gear 32 so that as the motor is operated rotary motion will be transmitted to the stem 29 at a greatly reduced speed over the speed of rotation of the motor shaft. While I have shown one 35 form of operating means for the valve 18, it is obvious however, that many forms of gear and power may be used to operate this valve, and I do not wish to limit myself to any specific gear or power but desire to use any 40 form of power available or any gear that may be needed in any specific instance, or even, if occasion requires, to operate valve 18 by hand.

The automatic pressure release valve 45 shown in detail in Fig. 4, comprises the case which has the valve proper 26, mounted therein between the connection of pipe 14 provided to form an outlet from the impregnating cylinder or retort 2, and the pipe 50 16 which returns to the liquid supply tank 1, and a spring 27 is provided to bear against this valve 26 to exert pressure to oppose the opening of this valve and consequently to oppose the passage of liquid from the outlet 55 pipe 14 to the return pipe 16. While the spring 27 is illustrated as a simple coil spring around the stem of the valve 26 to bear against the reverse side thereof and against the head of the case, it will be understood 60 that by changing this spring and substituting therefor a spring of a lighter or heavier gage, the valve 26 can be regulated to open at varied pressures, and here it might also be stated that it might be desirable to, in some uses, provide means

whereby the pressure of the spring 27 may be adjusted to accommodate various operating conditions and to give various settings thereto without the necessity of dismantling the parts to insert a new spring.

70

As is hereinbefore set forth, I have provided a motor 33 to control the valve 18, and the circuit wires from this motor are led to a generator 35, or to any other suitable source of electrical energy. Not only 75 is it desirable that the valve 18 be gradually closed to consequently gradually increase the pressure within the retort 2, but also it is desirable that some means be provided to automatically cut out the connection to the 80 motor so that the valve will not be given further actuation after a desired maximum pressure has been attained within the retort, and to accomplish this purpose I provide the diaphragm pressure switch, as better 85 shown in Fig. 5, which switch 36 is connected in one of the circuit wires to the motor 33 and is designed to automatically stop the motor when the maximum retort pressure has been accomplished. A pipe 37 90 is led from the retort chamber to connect with the diaphragm chamber 38, and in this way when pressure sufficiently strong to overcome the pressure of the spring 39 is accomplished in the retort, this pressure 95 will be transferred through the pipe 37 to the diaphragm chamber 38 and in consequence the switch arm 40 will be swung outwardly to break the switch connection.

In the accomplishment of the process, the 100 timber, ties, poles, paving blocks, etc., are loaded on trucks and run into the retort, or are otherwise placed therein, and the door 5 is closed into place and is secured to make the retort air and liquid tight. Steam 105 is admitted through the valve 19 and the pipe 20, passes through pipe 11 into branch pipes 12 and is uniformly distributed throughout the interior of the retort 2 through the openings 13. After the wood in 110 the retort 2 is heated to the proper temperature, generally about 250 degrees Fah., for the necessary time, generally from one to five hours, the valve 19 is closed to shut off the supply of steam and the steam contained in the retort 2 is blown away until the pressure in the retort is at or nearly at atmospheric pressure. The blow-off, not shown, is then closed and valve 25 in pipe 24 which leads to the vacuum pump is opened, 115 thus permitting the air, moisture, and steam within the retort to be drawn out of the retort 2 and passed away through the vacuum pump. This operation extracts the air and moisture from the wood leaving the 120 cells and pores thereof open and in proper condition to absorb the preserving liquid.

After a vacuum of from 22 to 25 or more inches of mercury has been maintained in the interior of the retort 2, for under or 130

dinary working conditions, from forty minutes to one hour, the valve 8 in the pipe 7 is opened and liquid flows from the supply tank 1 into the exhausted retort 2 to entirely fill this retort and completely submerge the wood contained therein to be treated. The valve 25 in the pipe 24 is then closed to cut off communication from the vacuum pump, valve 8 is closed to cut off communication from the liquid supply tank 1 to the retort 2 through the valve 7, valve 18 is opened, and pump 9 is started in operation. The mechanical arrangement which operates valve 18 is then set in operation so that the valve will be gradually closed, or care is taken by the operator to manually manipulate this valve to accomplish the gradual closing of the passage therethrough. The pump 9 takes liquid through the pipe 10 from the liquid supply tank 1, and forces this liquid through pipe 11 to be discharged through the openings 13 into all parts of the retort. As the retort has been filled through pipe 7, the further supply of liquid thereto through the pipe 11 causes the impregnating liquid to be forced through the retort 2 out through the plurality of branches in the pipe 14, thence through the pipe 17 and valve 18 back to the liquid-supply tank 1, the pressure of the spring in the valve 15 acting to close communication therethrough while the valve 18 is still open. As the valve 18 is gradually closed, the pressure in the retort is raised to the maximum pressure as desired.

It is preferable that the passage through valve 18 be made of triangular shape, as shown in Fig. 2, for the reason that when the pump is started, circulation begins and the full opening through the valve 18 allows the full volume of liquid supplied to the retort 2 to pass freely through the valve 18. As the area of outlet through valve 18 is gradually restricted due to the mechanical closing of the valve 18, there is a corresponding rise of pressure in the retort 2, since the velocity of the flow of the liquid is increased about as the square of its pressure. Therefore, to obviate the necessity of changing the speed of the gearing from the motor at frequent intervals to render the raising of the pressure in the retort 2 uniform and automatic, it is necessary that the valve moving at a uniform speed, restrict a relatively larger area of opening at the beginning of the operation and a gradually decreasing area as the velocity of liquid flow increases, due to the increasing pressure in the retort 2, and hence I make use of the triangular outlet.

When the maximum pressure in the retort 2 is attained, the liquid pressure acting on the diaphragm of the automatic switch 36 forces the switch arm 40 open, breaking the circuit contact, and the motor is thus auto-

matically stopped. The valve 18 will, by reason of the fact that the pressure in the retort will be maintained substantially constant and the circuit connections will thus be held open, stand at this point during the balance of the treating operation, and thus circulation will be continued and the pressure will be maintained substantially constant at the maximum for which the automatic switch has been set.

The pressure release valve 15 is set to discharge at or near the maximum pressure at which the retort 2 is operated, and thus act as a safety valve to relieve any excess of fluid over the volume that will be discharged through the restricted opening of the valve 18, which increases in the volume of fluid may at times be caused by variations in the speed of operation of the pump 9, and thus all danger of excessive or over pressure is obviated.

While I have herein shown one specific form of apparatus which is adaptable for the accomplishment of the process, and an apparatus which will carry out the steps thereof in proper order, it will be understood that changes in the apparatus may be made and may even be desirable under various operating conditions, therefore, I do not wish to limit myself to any particular arrangement of the apparatus, and further do not wish to be limited in so far as the process is concerned, except for such limitations as the claims may impart.

I claim:

1. The method of preserving wood which consists in treating the wood by the circulation of a preservative fluid in and through a retort in which the wood is placed and in and through an open circuit piping system to thus provide for elimination of free air from the retort.

2. The method of impregnating wood which consists in placing the wood in a container, filling the container with preservative liquid, injecting liquid into the container to be equally supplied in all parts, and discharging liquid from the container at different points to secure a flow through and circulation in all parts of the retort.

3. The method of impregnating wood which consists in placing the wood in a container, injecting liquid into the container at the bottom thereof to be equally supplied in all parts, discharging liquid from the container at the top thereof and at different points to secure an equal flow through and circulation in all parts of the container, and constricting the discharge to raise the pressure of liquid within the container.

4. The method of impregnating wood which consists in placing the wood in a retort, filling the retort with preservative liquid taken from a liquid supply, maintaining a constant supply and flow of liquid

under pressure into all parts of the retort, discharging liquid from the retort at different points to secure an equal flow through and circulation in all parts of the retort, 5 conducting the discharge liquid to the liquid supply, and agitating the liquid at the supply to be reinjected into the retort.

5. The method of impregnating wood which consists in placing the wood in a 10 retort, filling the retort with preservative liquid taken from a liquid supply, maintaining a constant supply and flow of liquid under pressure into all parts of the retort, discharging liquid from the retort at different points to secure an equal flow through 15 and circulation in all parts of the retort, conducting the discharge liquid to the liquid supply, agitating the liquid at the supply to be reinjected into the retort, gradually 20 constricting the discharge to thus raise the

pressure within the retort to a maximum, and maintaining this maximum pressure within the retort for a period of time to secure proper penetration of the liquid into the wood.

6. The method of preserving wood by the use of a preservative fluid constituting a plurality of chemical ingredients, which consists in submerging the wood in the fluid mixture and maintaining a continuous flow 30 of the fluid mixture from and to a fluid supply, and constantly mixing the preservative fluid at the fluid supply.

In testimony whereof I affix my signature in presence of two witnesses.

W. A. CECIL.

Witnesses:

ALLEN DEAN,  
RAYMOND MEYER.